



US007541129B2

(12) **United States Patent**  
**Koyama et al.**

(10) **Patent No.:** **US 7,541,129 B2**  
(45) **Date of Patent:** **Jun. 2, 2009**

(54) **ELECTROSTATIC IMAGE DEVELOPING TONER**

(75) Inventors: **Mikio Koyama**, Kunitachi (JP); **Kenji Hayashi**, Hachioji (JP); **Kazuya Isobe**, Hachioji (JP); **Yasuhiro Saita**, Hachioji (JP)

(73) Assignee: **Konica Minolta Business Machines Technologies, Inc.**, Tokyo (JP)

(\*) Notice: Subject to any disclaimer, the term of this patent is extended or adjusted under 35 U.S.C. 154(b) by 415 days.

(21) Appl. No.: **11/353,439**

(22) Filed: **Feb. 14, 2006**

(65) **Prior Publication Data**

US 2006/0188802 A1 Aug. 24, 2006

(30) **Foreign Application Priority Data**

Feb. 21, 2005 (JP) ..... 2005-043798

(51) **Int. Cl.**

**G03G 9/08** (2006.01)

(52) **U.S. Cl.** ..... **430/108.4**; 430/110.1; 430/124.3

(58) **Field of Classification Search** ..... 430/108.4, 430/124.3, 110.1, 137.14, 137.17

See application file for complete search history.

(56) **References Cited**

U.S. PATENT DOCUMENTS

4,642,281 A 2/1987 Kakimi et al.  
4,933,249 A \* 6/1990 Mikami ..... 430/123.5  
2003/0036013 A1 2/2003 Yamazaki et al.

FOREIGN PATENT DOCUMENTS

|    |             |         |
|----|-------------|---------|
| JP | 2000-214629 | 8/2000  |
| JP | 2001272813  | 5/2001  |
| JP | 2002-287405 | 10/2002 |
| JP | 2003-091101 | 3/2003  |

\* cited by examiner

Primary Examiner—Janis L Dote

(74) Attorney, Agent, or Firm—Lucas & Mercanti, LLP

(57) **ABSTRACT**

An electrostatic image developing toner comprising a binder resin and a colorant, wherein the toner contains a mixture of: (i) a compound represented by Formula (3); and (ii) a compound represented by Formula (1) and/or (2), wherein R<sub>1</sub> to R<sub>8</sub> each represent an alkyl group having 10 to 30 carbon atoms and X represents H or —CO—R<sub>9</sub>, wherein R<sub>9</sub> represents an alkyl group having 1-4 carbon atoms:



**17 Claims, 4 Drawing Sheets**

FIG. 1



FIG. 2



FIG. 3



FIG. 4



# ELECTROSTATIC IMAGE DEVELOPING TONER

## FIELD OF THE INVENTION

The present invention relates to an electrostatic image developing toner, more specifically, relates to an electrostatic image developing toner containing an ester compound having a specified structure.

## BACKGROUND OF THE INVENTION

Recently in the field of the image forming technology based on electrophotography such as copiers and printers, required has been a technology of a level which enables an accurate reproduction of a microdot image of 1200 dpi (in the present invention, "dpi" indicates the number of dots per 2.54 cm) in accordance with the development of the digital technology.

In order to faithfully reproduce the microdot image, miniaturization of the diameter of a toner particle has been studied, and attracted attention has been a chemical toner represented by a polymerization toner to which various types of controls can be applied in the manufacturing process, and, as a result, toner with a small diameter for faithfully reproducing the microdot image has been obtained (for example, see Patent Document 1).

On the other hand, as a method for fixing a toner image transferred on an image forming substance (also referred to as a transfer material) such as paper, a fixing method based on contact fixing, for example, a thermal roll fixing method and a thermal belt fixing method, is widely used. However, the contact fixing method tends to cause an offset problem in which melted toner adheres onto a heat member and the adhered toner is transferred to another image forming substance.

As the method to prevent the offset problem, for example, there has been a method to add a releasing property to the heat member by coating silicon oil on a surface of the heat member of a fixing device. However, the transfer material (image forming substance) coated with silicon oil becomes unrewritable with a writing tool such as a ball-point pen, and the transfer material may be contaminated by a volatile component contained in the silicon oil, both of which are not favorable for a business tool.

To cope with the above problem, development of an oil-less toner in which a releasing property is added to the toner particle itself has been carried out, and appeared has been a technology to add a fixing improver in the toner particle to provide the toner with a releasing property. To provide a releasing property, for example, an oil-less chemical toner containing a compound such as an ester compound of higher fatty acid having a long chain hydrocarbon group has been developed (for example, see Patent Documents 2, 3). The appearance of the toner containing the ester compound as the release agent has greatly contributed to the development of the oil-less image formation technology.

Recently, for the image formation technology based on the electrophotographic method, there has been a demand to reduce the electric consumption of printers or copiers in order to reduce the influence to the environment in association with the image formation and the business costs in the office. As one of the measures to achieve the above demand, a technology to lower the fixing temperature of such electrophotographic image compared to the current fixing temperature has attracted attention. Further, because of the characteristic that the required number of sheets can be printed at required time,

an image forming apparatus based on electrophotography has been extensively used in the field of short run printing.

However, when fixing was carried out at a lower temperature using the toner-containing the above ester compound, the formed toner image was found to have a tendency to easily peel from the transfer material. Further, when a large amount of printing was continuously carried out, for example, a several hundred-thousand-sheets of printing was repeated, the charge rising capability of the toner showed a tendency to degrade, accordingly, durability of the toner has been desired, by which the charge rising capability did not vary even when a large amount of image formation was repeated. As described above, there has been a demand to provide a property, which meets the new movements or the needs of the market, to an oil-less toner.

Patent Document 1: Japanese Patent Publication Open to Public Inspection (hereafter referred to as JP-A) No. 2000-214629 (see Paragraph 0061 and other paragraphs)

Patent Document 2: JP-A No. 2002-287405 (see Paragraph 0051 and other paragraphs)

Patent Document 3: JP-A No. 2003-91101 (see Paragraph 0208 and other paragraphs)

## SUMMARY OF THE INVENTION

An object of the present invention is to provide an electrostatic image developing toner which enables a wide range of fixable temperature in which sufficient adhesion of the toner image to the transfer material is attained where the toner image hardly peels from the transfer material and offset to another transfer material is avoided, even when the toner image is fixed at a surface temperature of the transfer material as low as 100°C.

Another object of the present invention is to provide an electrostatic image developing toner exhibiting an excellent durability which enables to maintain a stable charge rising capacity of the tone even after a large amount of copies, for example, several hundred-thousand-sheets of copies, are carried out.

One of the aspects of the present invention is an electrostatic image developing toner containing a binder resin and a colorant, wherein the toner comprises a mixture of: (i) a compound represented by Formula (3); and (ii) a compound represented by Formula (1) and/or (2):



wherein, R<sub>1</sub>, R<sub>2</sub> and R<sub>3</sub> each independently represent an alkyl group having 10 to 30 carbon atoms and the alkyl group may have a substituent;



wherein, R<sub>4</sub> and R<sub>5</sub> each independently represent an alkyl group having 10 to 30 carbon atoms and the alkyl group may have a substituent; and



Formula (3)



Formula (3)

wherein, X represents H or —CO—R<sub>9</sub>, R<sub>9</sub> represents an alkyl group having 1-4 carbon atoms, where the alkyl group may have a substituent, and R<sub>6</sub>, R<sub>7</sub> and R<sub>8</sub> each independently represent an alkyl group having 10 to 30 carbon atoms, where the alkyl group may have a substituent.

#### BRIEF DESCRIPTION OF THE DRAWINGS

FIG. 1 is a cross-sectional configuration view showing an example of an image forming apparatus used in the present invention.

FIG. 2 is a cross-sectional view showing an example of a fixing device (of a type using a pressure roller and a heat roller) used in the present invention.

FIG. 3 is a schematic view showing an example of the fixing device (of a type using a belt and the heat roller) used in the present invention.

FIG. 4 is a schematic-view showing an example of the fixing device (of a type using a soft roller and the heat roller) used in the present invention.

#### DESCRIPTION OF THE PREFERRED EMBODIMENTS

An aspect of the invention is an electrostatic image developing toner comprising a binder resin and a colorant, wherein the toner contains a mixture of:

- (i) a compound represented by Formula (3); and
- (ii) a compound represented by Formula (1) and/or (2):



Formula (1)

wherein, R<sub>1</sub>, R<sub>2</sub> and R<sub>3</sub> each independently represent an alkyl group having 10 to 30 carbon atoms and the alkyl group may have a substituent;



Formula (2)

wherein, R<sub>4</sub> and R<sub>5</sub> each independently represent an alkyl group having 10 to 30 carbon atoms and the alkyl group may have a substituent; and

10 wherein, X represents H or —CO—R<sub>9</sub>, R<sub>9</sub> represents an alkyl group having 1-4 carbon atoms, where the alkyl group may have a substituent, and R<sub>6</sub>, R<sub>7</sub> and R<sub>8</sub> each independently represent an alkyl group having 10 to 30 carbon atoms, where the alkyl group may have a substituent.

15 The electrostatic image developing toner of the present invention containing a mixture of: (i) a compound represented by Formula (3); and (ii) a compound represented by Formula (1) and/or (2) enables to provide an electrostatic image developing toner exhibiting an excellent adhesion of the toner image to the transfer material, where the toner image hardly peels from the transfer material, even when the toner image is fixed at a surface temperature of the transfer material as low as 100° C.

20 The present invention also enabled to provide of an electrostatic image developing toner exhibiting an excellent durability of the toner, by which high density images without fogging are obtained because the charge rising capacity of the toner is stable, even after a large amount of copies, for example, several hundred-thousand-sheets of copies, are carried out.

25 The present invention relates to a toner for developing an electrostatic image (hereafter, merely referred to as the toner) containing a mixture of a compound represented by Formula (3); and a compound represented by Formula (1) and/or (2).

30 The toner containing the mixture of a compound represented by Formula (3) and a compound represented by Formula (1) and/or (2) (hereafter, also referred to as “the mixture of ester compounds having specified structures” or merely as “the mixture”) was found to exhibit a robust fixing property in which the toner image hardly peel from the transfer material even when the toner image is fixed at a surface temperature of the transfer material as low as 100° C.

35 Namely, in the present invention, the mixture of ester compounds formed by reacting polycarboxylic acids and aliphatic alcohols each having a longer chain, as shown in Formulas (1)-(3), is incorporated in the toner particles.

40 It is not fully clear why the toner image formed by using the toner containing the mixture of ester compounds having the specified structures exhibits a robust fixing property, even when fixed at a lower temperature, however, it is assumed to be as follow:

45 The structure of the ester compound of the present invention is characterized by having two or three long chain hydrocarbon ester groups together with a short chain hydrocarbon ester group or a hydroxyl group. The presence of long chain hydrocarbon groups is assumed to have contributed to exhibit an excellent releasing property. Further, the presence of the long chain hydrocarbon groups is assumed to have contributed to exhibit a moderate affinity of the ester compound to the components of the toner particles, resulting in forming a microdomain structure since the ester compound is suitably dispersed in the toner particles due to the affinity of the long chain hydrocarbon groups to the toner components. The microdomain structure would have further improved the 50 releasing property of the toner.

55 The existence of a short chain aliphatic hydrocarbon ester group having 1-4 carbon atoms or a hydroxyl group in the

ester compound is assumed to have contributed to improve the adhesiveness of the toner to the transfer material as a result of forming a bond between the short chain aliphatic hydrocarbon ester group or the hydroxyl group with the cellulose contained in the paper used as a transfer material. The existence of the short chain aliphatic hydrocarbon ester group or the hydroxyl group commonly effects to deteriorate the releasing property, however, in the ester compound of the present invention, the plurality of long chain aliphatic hydrocarbon ester groups having higher affinity to the fixing roller would have oriented first to the roller, by which deterioration of releasing property is avoided.

Further, in the present invention, the fixing property at a lower fixing temperature is assumed to have improved because the temperature range of melting point of the ester compound is wider in the present invention since the mixture contains a plurality of ester compounds represented by Formula (3) and also represented by Formulas (1) or (2). Namely, when ester compounds having different number of carbon atoms are melted, the compound having a smaller number of carbon atoms melts first, by which the compound having a larger number of carbon atoms melts under its melting point, whereby the melting of the whole compound is accelerated.

Since these ester compounds steadily melts at a lower temperature, the melting of the whole the mixture of ester compounds is accelerated and the melted compound immediately and assuredly moves to the surface of each toner particle, whereby the releasing property is improved as well as the fixing property is improved. This effect is more notable for small diameter toners.

The charge rising capacity of the toner of the present invention was found to be stable even after a large amount of copies, for example, several hundred-thousand-sheets of copies, were carried out. This is assumed to be because, the mixture of the ester compounds has a structure in which the groups having strong affinity to water, for example, ester groups or hydroxyl groups, exist in the center part of the molecule. Namely, since the ester groups exist in the center part of the molecule near the quaternary carbon atom (representing a carbon atom which has no direct bond with a hydrogen atom), in a process to form particles in an aqueous medium, the ester compound is supposed to take a structure in which the quaternary carbon is oriented toward the water because the ester groups exist near the quaternary carbon atom. As a result, on the surface of the toner, the ester compounds exist with orienting the ester groups outside of the toner particle. Thus, toner particles having polar groups oriented outside of the toner are formed. The charge rising capability is improved due to the effect of the polar groups existing on the surface of the toner particles. Further, since the compounds represented by Formulas (1) and (2) each has an unsaturated bond in the molecule, rotation in the molecule is not allowed, resulting in enabling the hydrocarbon groups to be assuredly oriented in the molecule. Accordingly, these compounds are assumed to have a multiplier effect with the compound represented by Formula (3).

The present invention will be described in detail below.

The compounds represented by Formulas (1), (2) and (3) are ester compounds each of which is formed by reacting long chain aliphatic alcohols with a polycarboxylic acid, for example, a citric acid.



10 wherein, R<sub>1</sub>, R<sub>2</sub> and R<sub>3</sub> each independently represent an alkyl group having 10 to 30 carbon atoms and the alkyl group may have a substituent R<sub>1</sub>, R<sub>2</sub> and R<sub>3</sub> may have the same structure or may have different structures from each other.



wherein, R<sub>4</sub> and R<sub>5</sub> each independently represent an alkyl group having 10 to 30 carbon atoms and the alkyl group may have a substituent.



wherein, X represents H or —CO—R<sub>9</sub>, R<sub>9</sub> represents an alkyl group having 1-4 carbon atoms, where the alkyl group may have a substituent, and R<sub>6</sub>, R<sub>7</sub> and R<sub>8</sub> each independently represent an alkyl group having 10 to 30 carbon atoms, where the alkyl group may have a substituent.

Specifically, each of the ester compounds contains two or three long chain aliphatic hydrocarbon ester groups together with a short chain aliphatic hydrocarbon ester group or a hydroxyl group in the molecule. R<sub>1</sub>, R<sub>2</sub>, R<sub>3</sub>, R<sub>4</sub>, R<sub>5</sub>, R<sub>6</sub>, R<sub>7</sub>, R<sub>8</sub> and R<sub>9</sub> in the above formulas may have the same structure or may have different structures from each other. Alkyl groups of R<sub>1</sub>-R<sub>9</sub>, preferably have no substituent, however, when those groups have a substituent, preferable examples include a sulfonic acid group, a nitro group, an amino group, and a hydroxyl group.

As specific ester compounds, listed are, for example, the following compounds (1-1) to (1-7), (2-1) to (2-7) and (3-1) to (3-16):



-continued



-continued

(3-2)



-continued

(3-15)



(3-16)

The ester compound having the specified structure of the present invention can be prepared, for example, by a dehydration condensation of a polycarboxylic acid and long chain aliphatic alcohols each having 10-30 carbon atoms.

The mixture of the ester compounds having specific structures of the present invention contains a compound represented by Formula (3) as a main component mixed with an appropriate amount of a compound represented at least one of Formulas (1) and (2) as an additional component.

The mixture of the ester compounds having specific structures of the present invention preferably contains 50% by weight or more of a compound represented by Formula (3) and less than 50% by weight of a compound represented at least one of Formulas (1) and (2). The content of the compound represented by Formula (3) is more preferably 60-98% by weight and still more preferably 80-95% by weight.

In the mixture of ester compounds containing a compound represented by Formula (3) and a compound represented by at least one of Formulas (1) and (2), the difference between (i) the number of total carbon atoms in the compound represented by Formula (3) (as the main component) and (ii) the number of total carbon atoms in the compound represented by at least one of Formulas (1) and (2) (as the additional component) is preferably less than 10. The reason of this is not fully clear, however, it is assumed that, when two compounds exhibiting a large difference in total carbon numbers are mixed each other, the difference in solubility of the two compounds tends to become larger resulting in lowering the solubility of the mixture.

The content of the mixture of the ester compounds having the specified structures of the present invention is preferably 1-15% by weight and more preferably 3-12% by weight based on the total weight of the toner.

By controlling the content of the mixture of the ester compounds having the specified structures in the above described range, the toner can exhibit an excellent releasing property and an excellent electrostatic chargeability.

Next, the method for manufacturing the toner of the present invention will be described.

The toner of the present invention is preferably obtained by at least polymerizing a polymerizable monomer in an aqueous medium. This manufacturing method includes: (i) preparing resin microparticles by polymerizing polymerizable monomer by means of suspension polymerization, or of emulsion polymerization or miniemulsion polymerization in an aqueous medium added with an emulsion of required additive, (ii) adding microparticles of a resin which works as a chargeability control agent, if necessary, and (iii) flocculating or fusing the formed particles by adding a flocculant such as an organic solvent or a salt.

#### (Suspension Polymerization Method)

An example of the method of manufacturing the toner of the present invention is as follows: a chargeability control

resin is also added to the polymerizable monomer in which various types of component materials such as a colorant or a release agent according to the necessity and a polymerization initiator are added, and then the various types of component materials are dissolved or dispersed in the polymerizable monomer with a machine such as a homogenizer, a sand mill, a sand grinder, or an ultrasonic homogenizer. The polymerizable monomer with the various types of component materials dissolved or dispersed therein is dispersed in an aqueous medium containing a dispersion stabilizer into oil droplets of a desired size as a toner using a machine such as a homomixer or a homogenizer. Subsequently, the system is heated to carry out polymerization. After the reaction is completed, the dispersion stabilizer is removed from the resulting system, and then filtered, rinsed, and dried to prepare the toner of the present invention. The "aqueous medium" in the present invention represents that the water content in the medium is 50% by weight or more.

#### (Emulsion Polymerization Method)

Further, another method of manufacturing the toner of the present invention may include a method of preparing the toner by subjecting resin particles to salting-out/fusion-bonding in the aqueous medium. Listed as this method, although not specifically limited, may be methods disclosed in, for example, JP-A Nos. 5-265252, 6-329947, 9-15904. Namely, the toner of the present invention may be formed by the method in which a plurality of dispersion particles of the component materials such as resin particles and a colorant, or particles composed of a resin and a colorant and the like are subjected to salting-out, flocculation and fusion-bonding, specifically, after the particles are dispersed using these emulsifying agents in water, the resulting dispersion is added with a flocculating agent of the critical flocculation density or more to be subjected to salting-out, at the same time heat fusion-bonding at a temperature higher than the glass transition point of the formed polymer itself to form fused particles while gradually growing the particle diameter, and the diameter growing is stopped at the time when the intended particle diameter is acquired by adding a large amount of water, wherein the particles further being heated and stirred to control the shape of the particle surface to be flat and smooth, and then heated and dried in the state of containing water and fluidity. Incidentally, together with the flocculating agent, a solvent which is infinitely dissolvable to water such as alcohol may be added herein.

In the method of manufacturing the toner of the present invention, the preferably used method is that the mixture of the ester compounds having the specified structure is dissolved or dispersed in the polymerizable monomer followed by mechanically dispersing the monomer in an aqueous medium to be subjected to miniemulsion polymerizing and subsequently the formed composite resin particles and colorant particles are subjected to salting-out/fusion-bonding. When the mixture of the ester compounds having the specified structure is dissolved in the polymerizable monomer, the ester compound having the specified structure may be merely dissolved or may be dissolved after melting.

Further, in the method of manufacturing of the toner of the present invention, preferably employed is the process of subjecting the composite resin particles obtained by a multistage polymerization method and the colorant particles to salting-out/fusion-bonding.

Next, a preferable example of the method of manufacturing the toner (the emulsion aggregation method) will be described in detail.

This manufacturing method may include the following processes: (1) a dissolution/dispersion process to dissolve or disperse the mixture of the ester compounds having the specified structure in a radical polymerizable monomer; (2) a polymerization process to prepare a dispersion of resin particles; (3) a fusion-bonding process to fuse the resin particles and colorant particles in an aqueous medium to obtain colored particles (association particles); (4) a cooling process to cool down the dispersion of the toner particles; (5) a cleaning process to solid-liquid separate the toner particles from the cooled dispersion of the toner particles and to remove the surfactant from the toner particles; (6) a dry process to dry the cleaned toner particles; and, if necessity, (7) a process to add an external additive to the dried toner particles.

Each of the above processes will now be described below.

[Dissolution/Dispersion Process]

This process is a process to dissolve or disperse the mixture of the ester compounds having the specified structure in the radical polymerizable monomer to prepare a radical polymerizable monomer solution containing the mixture of the ester compounds having the specified structure.

[Polymerization Process]

In a preferred example of the polymerization process, liquid droplets of the radical polymerizable monomer solution containing the mixture of the ester compounds having the specified structure are formed by applying mechanical energy in an aqueous medium in which added is a surfactant of not more than the critical micelle concentration (CMC), and the polymerization is carried out in each liquid droplets by adding a water-soluble radical polymerization initiator. Incidentally, an oil soluble polymerization initiator may be contained in the liquid droplets. In such a polymerization process, a treatment of forcibly emulsifying (forming liquid droplets) by applying mechanical energy is required. The means of applying the mechanical energy may include the means of applying the strong agitation or ultrasonic vibration energy such as a homo-mixer, ultrasonic waves, and Manton-Gaulin.

With the polymerization process, resin particles containing the mixture of the ester compounds having the specified structure and binder resin can be obtained. The resin particles may be colored particles or uncolored particles. The colored resin particles are obtained by subjecting the monomer composition containing a colorant to the polymerization treatment. When the uncolored resin particles are used, a dispersion of the colorant particles is added to the dispersion of the resin particles in the fusion-bonding process described below, wherein the resin particles and the colorant particles are fusion-bonded to form the toner particles.

[Fusion-Bonding Process]

As the method of fusion-bonding in the fusion-bonding process, the salting-out/fusion-bonding method using the resin particles (colored or uncolored resin particles) obtained from the polymerization process is preferred. Further, in the fusion-bonding process, in addition to the resin particles and colorant particles, release agent particles and particles of an internal additive such as a charge control agent can be fusion-bonded.

In the fusion-bonding process, the "aqueous medium" is referred to as that mainly of water (50% by weight or more). Listed as the components other than water may be organic solvents which dissolve in water including, for example, methanol, ethanol, isopropanol, butanol, acetone, methyl-ethyl ketone, tetrahydrofuran. Of these, specifically preferable are alcohol-series organic solvents such as methanol, ethanol, isopropanol, butanol which do not dissolve the resin.

The colorant particles can be prepared by dispersing a colorant in the aqueous medium. The dispersion treatment of the colorant is carried out in the state where the concentration of the surfactant is not less than the critical micelle concentration (CMC) in water. Although the homogenizer used for the colorant dispersion treatment is not specifically limited, preferably listed are the ultrasonic homogenizer, mechanical homogenizer, pressure homogenizers such as Manton-Gaulin and pressure type homogenizer, sand grinder, media type homogenizers such as GETZMANN MILL and diamond fine mill. Further, the surfactant used herein may include that similar to the surfactant as described above. Incidentally, the colorant (particles) may be subjected to surface modification. The surface modification method of the colorant is as follows: the colorant is dispersed in a solvent and the surface modification agent is added, and then the resulting system is reacted by raising the temperature thereof. After the reaction is completed, the colorant is filtered and repeatedly cleaned with the same solvent, and then is dried to obtain a colorant (pigment) treated with the surface modification agent.

The salting-out/fusion-bonding method which is the preferred method is the process that a salting-out agent which is a metal salt such as an alkali metal salt or an alkaline earth metal salt is added as the flocculating agent of the critical flocculation concentration or more in water in which resin particles and colorant particles exist, and subsequently the resulting solution is heated to a temperature which is not lower than the glass transition point of the resin particle and also not lower than the melting peak temperature (°C.) of the mixture of the ester compounds having the specified structure to conduct salting-out, at the same time carrying out fusion-bonding. In this process, a method of effectively carrying out fusion-bonding by adding the organic solvent which is infinitely dissolvable in water to practically lower the glass transition temperature of the resin particle may be adopted. Examples of the alkali metal salt and alkaline earth metal salt usable for the salting-out agents include: salts of alkali metals, for example, lithium, potassium and sodium; and salts of alkaline earth metals, for example, magnesium, calcium, strontium and barium, of these preferable are salts of potassium, sodium, magnesium, calcium and barium. Listed as components of the salt may be, for example, chlorine salt, bromine salt, iodine salt, carbonate and sulfate. Further, listed as the organic solvents infinitely dissolvable in water may be, for example, methanol, ethanol, 1-propanol, 2-propanol, ethylene glycol, glycerin, acetone, and preferably the alcohols of methanol, ethanol, 1-propanol, 2-propanol, having not more than 3 carbon atoms, and specifically preferably 2-propanol.

The above salting-out step and the fusion-bonding step may also be carried out separately.

When the fusion-bonding is carried out by salting-out/fusion-bonding, a period of time for leaving the system after the salting-out agent is added is preferably as short as possible. Although the reason thereof is not clear, the following problems occur that depending on the leaving period of time after salting out, the flocculation state of the particles varies, because the particle distribution is unstable and the surface property of the fusion-bonded toner varies. Further, the temperature at which the salting-out agent is added is preferably not higher than the glass transition temperature of the resin particle. The reason thereof is that when the temperature at which the salting-out agent is added is not lower than the glass transition temperature of the resin particle, the salting-out/fusion-bonding of the resin particle proceed fast while the particle diameter cannot be controlled, so that the large diameter particles tends to be disadvantageously generated. The addition temperature may be not higher than the glass transi-

## 13

tion temperature of the resin, however, generally in the range of 5-55° C., and preferably 10-45° C.

In the present invention, the salting-out agent is added at the temperature not higher than the glass transition temperature of the resin particle, and then the temperature is raised as fast as possible to heat to the temperature which is not lower than the glass transition temperature of the resin particle as well as not lower than the melting peak temperature (° C.) of the mixture of the ester compounds having the specified structure. The period of time while the temperature is increase is preferably less than one hour. Further, the temperature raising is preferably carried out quickly, and the temperature raising speed is preferably 0.25° C./min or more. The maximum temperature raising rate is not specifically limited, however, when the temperature is immediately increased, the salting-out rapidly proceeds and the particle diameter may become difficult to be controlled, and thereby it is preferably 5° C./min or less. With this fusion-bonding process, a dispersion of the association particles (toner particles) containing the resin particles and any other particles being subjected to salting-out/fusion-bonding can be obtained.

The glass transition temperature of the resin particle and the melting peak temperature of the ester compound having the specified structure can be measured by using DSC-7 (differential scanning calorimeter manufactured by Perkin Elmer, Inc.) and TAC7/DX (thermal analysis controller manufactured by Perkin Elmer, Inc.). The analysis procedure includes precise weighing a toner to be 4.5-5.0 mg to two places of decimals; enclosing the toner into an aluminum pan (Kit No. 0219-0041) and setting the pan on the sample-holder; and preparing a blank aluminum pan as a reference. The measurement conditions are as follows: the measurement temperature range of 0-200° C., the temperature increasing speed of 10° C./min and the temperature decreasing speed of 10° C./min. The temperature control is conducted so as to be 1st heating-1st cooling-2nd heating, and the analysis is based on the data in the 2nd heating. The glass transition temperature is the temperature at the intersection point of (1) the extension line of a base line before the endothermic peak temperature of the resin particle and (2) the tangential line giving the maximum inclination between the foot and the top of the endothermic peak. The melting peak temperature is indicated by a peak top temperature of the endothermic peak of the ester compound.

[Cooling Process]

This process is a process of subjecting the dispersion of the colored particles to the cooling treatment (quick cooling treatment). The condition of the cooling treatment is to cool at a cooling rate of 1-20° C./min. The method of the cooling treatment, although it is not specifically limited, may include a method of cooling by introducing a cooling medium from outside of a reaction container and a method of cooling by directly charging cool water into the reaction system.

[Solid-Liquid Separation and Cleaning Process]

In the solid-liquid separation and cleaning process, the following treatments are applied: a solid-liquid separation treatment of subjecting the colored particles to solid-liquid separation from the dispersion of the colored particles having been cooled down to a prespecified temperature in the above process; and a cleaning treatment of removing deposits such as the surfactant and the salting-out agent from a toner cake (an aggregation substance with a cake-shape) having been subjected to solid-liquid separation. Herein, the filter treatment method, which is not specifically limited, may include

## 14

the methods such as the centrifugal separation method, vacuum filtration method using Nutsche, and the filter method using a filter press.

[Drying Process]

This process is a process of subjecting the toner cake having been subjected to the cleaning treatment to the dry treatment to obtain dried colored particles. Listed as the dryer used in this process may be, for example, a spray dryer, a vacuum-freeze dryer, and a decompression dryer, and it is preferable to use a stationary rack-dryer, a movable rack-dryer, a fluidized dryer, a rolling dryer, an agitation dryer and other dryers. The water content of the dried colored particle is preferably 5% by weight or less, more preferably 2% by weight or less. Incidentally, when the toner particles having been subjected to the dry treatment are agglomerated with a weak intermolecular force among the particles, the agglomeration may be subjected to a powder treatment. Herein, mechanical type of powder machines such as a jet-mill, HENSCHEL MIXER, a coffee mill, a food processor may be used as the powder treatment machine.

[External Additive Treatment Process]

This process is a process of manufacturing the toner by mixing an external additive in the dried toner particles according to the necessity.

As the mixer for the external additive, mechanical type of mixers such as a HENSCHEL MIXER and a coffee mill may be used.

The volume median diameter ( $D_{v50}$ ) of the toner of the present invention is preferably 3-9  $\mu\text{m}$ . The toner of the present invention preferably has a CV value in volume particle size distribution of the toner of not more than 20%.

A CV value in volume based particle size distribution represents a degree of dispersion in volume particle size distribution of toner particles, and is defined by the following equation. The smaller a CV value is, the sharper the particle size distribution is; which means that the diameter of toner particles is uniform.

$\text{CV value} = (\text{standard deviation in volume particle size distribution}) / (\text{volume median diameter } (D_{v50})) \times 100$ . The volume median diameter and the CV value of the toner are measured and calculated by using COULTER MULTISIZER III (produced by Beckman Coulter Inc.), connected with a computer system (produced by Beckman Coulter Inc.) for data processing.

Measurement is carried out as follows: A surfactant solution is prepared, for example, by 10 times diluting a commercially available neutral detergent containing a surfactant with pure water. 20 ml of the surfactant solution is mixed with 0.02 g of toner. After making the toner blended with the surfactant solution, the mixture is subjected to an ultrasonic dispersion for one minute to obtain a toner dispersion. The toner dispersion is then poured, using a pipette, in a beaker containing ISOTON II (diluent; produced by Beckman Coulter Inc.) placed in a sample stand, until the content shown in the monitor increased to 5% by weight. The count number of particles is set at 30,000 and a 50  $\mu\text{m}$  aperture is used.

The toner of the present invention can be used as a black toner or a colored toner.

The compounds (a binder resin, a colorant, a release agent, a charge control agent, an external additive and a lubricant) which constitutes the toner of the present invention will now be explained.

(Binder Resin)

Examples of a polymerizable monomer forming the binder resin include: styrenes, for example, styrene, o-methylsty-

rene, m-methylstyrene, p-methylstyrene,  $\alpha$ -methylstyrene, p-chlorostyrene, 3,4-dichlorostyrene, p-phenylstyrene, p-ethylstyrene, 2,4-dimethylstyrene, p-tert-butylstyrene, p-n-hexylstyrene, p-n-octylstyrene, a p-n-nonylstyrene, p-n-decylstyrene, and p-n-dodecyl styrene, and derivatives thereof; methacrylate derivatives, for example, methyl methacrylate, ethyl methacrylate, n-butyl methacrylate, isopropyl methacrylate, isobutyl methacrylate, t-butyl methacrylate, n-octyl methacrylate, 2-ethylhexyl methacrylate, stearyl methacrylate, lauryl methacrylate, phenyl methacrylate, diethylaminoethyl methacrylate and dimethylaminoethyl methacrylate; acrylate derivatives, for example, methyl acrylate, ethyl acrylate, isopropyl acrylate, n-butyl acrylate, t-butyl acrylate, isobutyl acrylate, n-octyl acrylate, 2-ethylhexyl acrylate, stearyl acrylate, lauryl acrylate and phenyl acrylate; olefins, for example, ethylene, propylene, and isobutylene; halogen-containing vinyls, for example, vinyl chloride, vinylidene chloride, vinyl bromide, and vinyl fluoride and vinylidene fluoride; vinyl esters, for example, vinyl propionate, vinyl acetate and vinyl benzoate; vinyl ethers, for example, vinyl methyl ether and vinyl ethyl ether; vinyl ketones, for example, vinyl methyl ketone, vinyl ethyl ketone and vinyl hexyl ketone; N-vinyl compounds, for example, N-vinylcarbazole, N-vinyl indole, and N-vinyl pyrrolidone; vinyl compounds, for example, vinyl naphthalene and vinyl pyridine; and acrylic acid or methacrylic acid derivatives, for example, acrylonitrile, methacrylonitrile and acrylamide. These vinyl monomers may be used alone or may be used in combination.

Moreover, it is still more preferable to use a polymerizable monomer having an ionically dissociable group in combination with a polymerizable monomer which constitutes the resin. For example, preferable are monomers having, for example, a carboxyl group, a sulfonic acid group, and a phosphate group as the composition group of a monomer. Specific examples of the monomer include: acrylic acid, methacrylic acid, maleic acid, itaconic acid, cinnamic acid, fumaric acid, maleic acid mono-alkyl ester, itaconic acid mono-alkyl ester, styrene sulfonic acid, allylsulfosuccinic acid, 2-acrylamide-2-methylpropanesulfonic acid, acid phosphoxyethyl methacrylate, 3-chloro-2-acid phosphoxypropyl methacrylate.

Further, polyfunctional vinyls may be used to form a resin having a cross-linking structure, example of the polyfunctional vinyl including: divinylbenzene, ethyleneglycol dimethacrylate, ethyleneglycol diacrylate, diethyleneglycol dimethacrylate, diethyleneglycol diacrylate, triethyleneglycol dimethacrylate, triethyleneglycol diacrylate, neopentylglycol dimethacrylate and neopentylglycol diacrylate.

These polymerizable monomer can be polymerized using a radical polymerization initiator. In this case, an oil soluble polymerization initiator can be used in a suspension polymerization method. Examples of the oil soluble polymerization initiator include: azo or diazo polymerization initiators, for example, 2,2'-azobis-(2,4-dimethylvaleronitrile), 2,2'-azobis-isobutyronitrile, 1,1'-azobis-(cyclohexane-1-carbonitrile), 2,2'-azobis-4-methoxy-2,4-dimethylvaleronitrile and azobisisobutyronitrile; and peroxide polymerization initiators or polymer polymerization initiators having a peroxide group as a side chain, for example, benzoyl peroxide, methyl-ethyl-ketone peroxide, diisopropyl peroxycarbonate, cumene hydroperoxide, t-butyl hydroperoxide, di-t-butyl peroxide, dicumyl peroxide, 2,4-dichloro benzoyl peroxide, lauroyl peroxide, 2,2-bis-(4,4-t-butyl peroxy)cyclohexyl propane and tris(t-butyl peroxy)triazine.

When using an emulsion polymerization method, a water-soluble radical polymerization initiator can be used. Examples of a water-soluble polymerization initiator include: persulfates, for example, potassium persulfate and ammonium

persulfate; azobis-aminodipropane acetate; azobis-cyanovaleic acid and its salt; and hydrogen peroxide.

(Colorant)

The colorant used in the present invention may be known inorganic or organic colorants. Specific colorants are listed below.

As the black colorant, for example, the carbon blacks such as furnace black, channel black, acetylene black, thermal black, and lampblack, and also the magnetic powders such as magnetite and ferrite are used.

Listed as the colorant for magenta or red include, for example: C. I. Pigment Red 2, C. I. Pigment Red 3, C. I. Pigment Red 5, C. I. Pigment Red 6, C. I. Pigment Red 7, C. I. Pigment Red 15, C. I. Pigment Red 16, C. I. Pigment Red 48:1, C. I. Pigment Red 53:1, C. I. Pigment Red 57:1, C. I. Pigment Red 122, C. I. Pigment Red 123, C. I. Pigment Red 139, C. I. Pigment Red 144, C. I. Pigment Red 149, C. I. Pigment Red 166, C. I. Pigment Red 177, C. I. Pigment Red 178 and C. I. Pigment Red 222.

Listed as the colorant for orange or yellow include, for example: C. I. Pigment Orange 31, C. I. Pigment Orange 43, C. I. Pigment Yellow 12, C. I. Pigment Yellow 13, C. I. Pigment Yellow 14, C. I. Pigment Yellow 15, C. I. Pigment Yellow 17, C. I. Pigment Yellow 93, C. I. Pigment Yellow 94, C. I. Pigment Yellow 138.

Listed as the colorant for green or cyan include, for example: C. I. Pigment Blue 15, C. I. Pigment Blue 15:2, C. I. Pigment Blue 15:3, C. I. Pigment Blue 15:4, C. I. Pigment Blue 16, C. I. Pigment Blue 60, C. I. Pigment Blue 62, C. I. Pigment Blue 66, C. I. Pigment Green 7.

Incidentally, these colorants may be used alone or may be used in combination of two or more of them, according to the necessity. The adding amount of the colorant is set to 1-30% by weight, and preferably in the range of 2-20% by weight, based on the total weight of the toner.

(Release Agent)

The release agent used in the present invention preferably contains the mixture of the ester compounds having the specified structure. The content of the mixture of the ester compounds having the specified structure is 1-15% by weight, and preferably 3-12% by weight, based on the total weight of the toner to obtain favorable results.

(Charge Control Agent)

In the toner of the present invention, a charge control agent may be added according to the necessity. As the charge control agent, known compounds may be used, specific examples of which include: a nigrosin dye, a metal salt of naphthenic acid or higher fatty acid, an alkoxylated amine, a quaternary ammonium chloride, an azo metal-complex, a salicylate metal salt or its metal-complex. Listed as the metal to be contained therein are, for example, Al, B, Ti, Fe, Co, Ni. Specifically preferable compound as a charge control agent is the metal-complex compound of benzilic acid derivatives. Incidentally, when the content of the charge control agent is 0.1-20.0% by weight based on the total weight of the toner, favorable results may be obtained.

(External Additive)

An external additive may be added and used in the toner particles for the purpose of improving the fluidity, charge property, cleaning property and for other purposes. The external agent is not specifically limited and various types of inorganic particles, organic particles, and lubricants may be used.

As the inorganic particles, known particles may be used. More specifically, particles of silica, titania, alumina, stron-

tium titanate may preferably be used. These inorganic particles that are subjected to the hydrophobic treatment may be used according to the necessity. Listed as the specific silica particles may be, for example, the commercially available products manufactured by Nippon Aerosil Co., Ltd., for example, R-805, R-976, R-974, R-972, R-812 and R-809; HVK-2150, H-200 manufactured by Hoechst AG; the commercially available products manufactured by Cabot Corp. such as TS-720, TS-530, TS-610, H-5 and MS-5.

Listed as the titania particles may be, for example, the commercially available products manufactured by Nippon Aerosil Co., Ltd. such as T-805, T-604; the commercially available products manufactured by Tayca Co., Ltd. such as MT-100S, MT-100B, MT-500BS, MT-600, MT-600SS, JA-1; the commercially available products manufactured by Fuji Titan Co., Ltd. such as TA-300SI, TA-500, TAF-130, TAF-510, TAF-510T; the commercially available products manufactured by Idemitsu Kosan Co., Ltd. such as IT-S, IT-OA, IT-OB, IT-OC and the like.

Listed as the alumina particles may be, for example, commercially available products manufactured by Nippon Aerosil Co., Ltd. such as RFY-C, C-604; the commercially available product manufactured by Ishihara Sangyo Kaisha Ltd. such as TTO-55 and the like.

Further, as the organic particles, those having a number average primary particle diameter of about 10 through 2000 nm with a spherical shape may be used. More specifically, homopolymers such as styrene and methyl methacrylate and their copolymer may be used.

The adding amount of these external additives is preferably 0.1 through 10.0% by weight based on the total weight of the toner. As the method of adding the external additive, various types of known mixers may be used such as, a turbular mixer, a HENSCHEL MIXER, a NAUTER MIXER, and a V-type mixer.

In the toner of the present invention, a lubricant may be mixed and used in the toner particles for the purpose of increasing the cleaning property and transfer property according to the necessity. Listed as the lubricant may be, for example, the metal salts of higher fatty acid such as the salts of zinc stearate, aluminum stearate, copper stearate, magnesium stearate, calcium stearate; the salts of zinc oleate, manganese oleate, iron oleate, copper oleate, magnesium oleate; the salts of zinc palmitate, copper palmitate, magnesium palmitate, calcium palmitate; the salts of zinc linoleate, calcium linoleate; the salts of zinc ricinoleate, calcium ricinoleate.

The adding amount of these lubricants is preferably 0.1 through 10.0% by weight based on the total weight of the toner. As the method of adding the lubricant, various types of known mixers may be used such as a turbular mixer, a HENSCHEL MIXER, a NAUTER MIXER, and a V-type mixer.

The toner of the present invention may be used as a mono-component developer or a two-component developer. When used as the mono-component developer, the toner may be formed as a magnetic mono-component developer in which magnetic particles of about 0.1 through 0.5  $\mu\text{m}$  is contained or may be used as a non-magnetic mono-component developer. Further, the toner may be used as the two-component developer by mixing with a carrier. In this case, as the magnetic particles of the carrier, known materials represented by iron-containing magnetic particles such as iron, ferrite, and magnetite may be used, of these, specifically preferable is the ferrite particle or the magnetite particle. The volume median diameter ( $D_{v50}$ ) of the above magnetic particles is preferably 15-100  $\mu\text{m}$ , and more preferably 20-80  $\mu\text{m}$ .

The median diameters ( $D_{v50}$ ) of the carrier particles are determined by using a laser diffraction particle diameter distribution meter "HELOS" (manufactured by Sympatec GmbH).

As the carrier, a coating carrier in which the magnetic particles are further coated with a resin, or a so-called resin dispersion type carrier in which the magnetic particles are dispersed in a resin is preferable. The resin composition for coating is not specifically limited. Examples of the resin for coating magnetic particles include: an olefin resin, a styrene resin, a styrene-acrylic resin, a silicon-containing resin, an ester resin or a fluorine-containing polymer resin. The resin for dispersing magnetic particles is not specifically limited and known resins may be used including, for example, a styrene-acrylic resin, a polyester resin, a fluorine-containing resin and a phenol resin.

Further, the mixing ratio of the carrier to the toner is preferably in the range of carrier:toner=1:1 through 50:1 in weight ratio.

The toner of the present invention is preferably used in an image forming apparatus based on the contact fixing method in which a transfer material having thereon a toner image is passed between heat members composing a fixing device to fix the image.

An image forming method using the toner of the present invention comprises: developing a latent image with a toner of the present invention so as to form a toner image.

Moreover, the image forming method further comprising fixing the toner image on an image forming material by passing between a first rotating member and a second rotating member, wherein at least one of the first and second rotating members gives heat to the toner image.

More specifically, the first rotating member is a roller and is provided with a heat source inside of the roller.

Even more specifically, the second rotating member includes a roller or an endless belt.

The image forming apparatus and the fixing device will be described below.

FIG. 1 is a cross-sectional view showing an example of an image forming apparatus used in the present invention.

In FIG. 1, 20Y (20M, 26C, 20Bk) represents a image forming unit, 21Y (21M, 21C, 21Bk) represents a photosensitive drum, 22Y (22M, 22C, 22Bk) represents a scorotron charger, 23Y (23M, 23C, 23Bk) represents an optical system for exposure, 24Y (24M, 24C, 24Bk) represents a developer, 25Y (25M, 25C, 25Bk) represents a cleaning device, 34Y (34M, 34C, 34Bk) represents a transfer device, 40 represents a fixing device, 115 represents a transfer material conveying belt, 160 represents a conveying device and P represents a transfer material.

The image forming apparatus illustrated in FIG. 1 will now be explained.

In the image forming unit shown in FIG. 1, four image forming units 20Y, 20M, 20C and 20Bk are provided along the transfer material conveying belt 115.

Each image forming unit includes: a photosensitive drum 21Y (21M, 21C, 21Bk), a scorotron charger 22Y (22M, 22C, 22Bk), an optical system for exposure 23Y (23M, 23C, 23Bk), a developer 24Y (24M, 24C, 24Bk) and a cleaning device (a cleaning means) 25Y (25M, 25C, 25Bk), and each toner image formed on each photosensitive drum (21Y, 21M, 21C, 21Bk) is sequentially transferred onto a transfer material P (for example, a transfer sheet and an OHP sheet) which is synchronously conveyed to form a superimposed color image.

A transfer material P is conveyed by the transfer material conveying belt 115 and then separated from the conveying belt with the aid of the AC static eliminator 161 and separating claw 210 which intermittently appears on the conveying device 160.

After passing through the conveying device 160, the transfer material P is sent to the fixing device (fixing means) 40 and wedged at the nip T formed between the heating roller 41 and the pressing roller 42 where heat and pressure are applied to fix the superimposed color image formed on the transfer material P and then discharged out of the apparatus.

The exposure device may be equipped with a scanning optical system employing semiconductor laser or a solid state scanner, for example, LED and a liquid crystal shutter.

As the material for the transfer material conveying belt 115, employed are polymer films, for example, polyimide and polycarbonate, and PVDF or electro conductive rubbers prepared by adding conductive fillers such as carbon black into synthetic rubbers such as silicone rubber or fluorine-containing rubber. The shape of the belt may be drum-like or belt-like, however, preferable is belt-like in view of the flexibility in device designing.

The surface of the transfer image conveying belt 115 is preferably moderately roughened. By roughening the surface of the belt so as to exhibit a 10 points surface roughness Rz of 0.5-2  $\mu\text{m}$ , the contact between the transfer material and the belt is improved and the movement of the transfer material on the belt is suppressed resulting in improving the transferability of the toner image from the photosensitive drum to the transfer material.

The transfer material used in the present invention is a support body for keeping the toner image, which is generally called as an image support body, a transfer body or a transfer sheet. More specifically, different types of transfer materials may be listed including plain papers from thin paper to thick paper, fine-quality paper, printing paper such as art paper and coated paper, Japanese paper and postcard paper which are commercially available, plastic film for OHP, and cloth, but the transfer material is not limited thereto.

FIG. 2 is a cross-sectional view showing an example of the fixing device 10 (a type of using a pressure roller and a heat roller) used in the present invention.

The fixing device 10 shown in FIG. 2 contains a heat roller 71 and a pressure roller 72 abutting the heat roller 71. Incidentally, in FIG. 2, reference numeral 17 denotes a toner image formed on the transfer material P (transfer sheet).

The heat roller 71 contains a coating layer 82 made of a fluorocarbon resin or an elastic body formed on a surface of a cored bar 81, the heat roller 71 further containing a heat member 75 made of a linear heater.

The cored bar 81 is composed of a metal and the inner diameter thereof is preferably 10-70 mm. The metal composing the cored bar 81 is not specifically limited, and such metals may be listed including, for example, iron, aluminum, copper or alloys of these metals.

The wall thickness of the cored bar 81 is preferably 0.1-15 mm, which is determined considering the balance between the requirement of energy saving (making the wall thinner) and the strength (depending on the component materials). For example, in order to keep the strength equivalent to that of the cored bar made of 0.57 mm thickness iron by the cored bar made of aluminum, the thickness of 0.8 mm is required.

As the fluorocarbon resin composing a surface of the coating layer 82, for example; PTFE (polytetrafluoroethylene) and PFA (tetrafluoroethylene-perfluoroalkylvinylether copolymer) may be listed.

The thickness of the coating layer 82 made of fluorocarbon resin is preferably 10-500  $\mu\text{m}$ , and more preferably 20-400  $\mu\text{m}$ .

When the thickness of the coating layer 82 containing fluorocarbon resin is less than 10  $\mu\text{m}$ , the function as the coating layer cannot be adequately performed, so that the durability as the fixing device cannot be assured. On the other hand, the surface of the coating layer over 500  $\mu\text{m}$  tends to have bruises due to paper powders, and the toner or other materials adheres at the bruise portions, causing the problem of image staining.

Further, as the elastic body composing the coating layer 82, a silicon rubber and a silicon sponge rubber having high heat resistance, for example, LTV, RTV and HTV are preferably used.

An Asker C hardness of the elastic body composing the coating layer 82 is preferably less than 80°, and more preferably less than 60°.

Further, the thickness of the coating layer 82 made of the elastic body is preferably 0.1-30 mm, and more preferably 0.1-20 mm.

As the heat member 75, a halogen heater is preferably used.

The pressure roller 72 contains a coating layer 84 made of an elastic body formed on a surface of a cored bar 83. The elastic body composing the coating layer 84 is not specifically limited, and various types of soft rubbers and sponge rubbers, for example, polyurethane rubber and silicon rubber are usable. Silicon rubber or silicon sponge rubber are preferably used as a material used for the coating layer 84.

Further, the thickness of the coating layer 84 is preferably 0.1-30 mm, and more preferably 0.1-20 mm.

Further, the fixing temperature (the surface temperature of the heat roller 10) is preferably 70-210° C., and the fixing linear velocity is preferably 80-640 mm/sec. The nip width of the heat roller is preferably 8-40 mm, and more preferably 11-30 mm.

Incidentally, the heat roller may be coated with a silicon oil of not more than 0.3 mg per print, or may be used oil-less.

FIG. 3 is a schematic view showing an example of the fixing device (a type using a belt and a heat roller).

The fixing device 10 shown in FIG. 3 is a type using a belt and the heat roller for keeping the nip width, wherein the key section contains a fixing roller 601 and a seamless belt 11, a pressure pads (pressure members) 12a, 12b which are pressed against the fixing roller 601 via the seamless belt 11, and a lubricant supplying member 40. B represents the rotation direction of the fixing roller 601.

The fixing roller 601 contains a heat resistant elastic body layer 10b and a releasing layer (heat resistant resin layer) 10c which are formed around a metal core (cylindrical cored bar) 10a, wherein inside the core 10a is provided with the halogen lamp 14 as the heat source. The temperature of a surface of the fixing roller 601 is measured with the temperature sensor 15, and the halogen lamp is feedback-controlled by a temperature controller not shown in response to the measured signal, whereby the surface of the fixing roller 601 is controlled so that the temperature thereof is constant. The seamless belt 11 is contacted as to be wound by a prespecified angle relative to the fixing roller 601 to form a nip section.

Inside the seamless belt 11 is provided with a pressure pad 12 having a low friction layer on a surface thereof in the state of being pressed against the fixing roller 601 via the seamless belt 11. The pressure pad 12 contains the pressure pad 12a to which a strong nip pressure is applied and the pressure pad 12b to which a weak nip pressure is applied, the pressure pads 12a, 12b being held by a holder 12c made of metal or other materials.

The holder 12c is further mounted with a belt-travel guide so that the seamless belt 11 can slide and rotate smoothly. Because the belt-travel guide chafes against an inner surface of the seamless belt 11, a member for the belt-travel guide is desired to have a lower friction coefficient and also has a low heat conduction in order not to take the heat away from the seamless belt 11. As a specific example of the material of the seamless belt, polyimide is preferably used.

The lubricant supplying member 40 includes a lubricant reservoir 41 and a lubricant transmission controlling film 42. The lubricant reservoir 41 has many continuous pores, and, for example, felt or sponge is preferably used. The lubricant reservoir 41 is impregnated with lubricant including silicone oil and fluorine-containing oil. The lubricant permeation controlling film 42 has many continuous pores, and, for example, a stretched fluorine-containing resin film is preferably used. In order to ensure the peeling of transfer materials from the fixing roller 601, a peeling member 20 as a supplementary member for the peeling may be provided on downstream of the nip section of the fixing roller 601. The peeling member 20 is held by holder 20b so that a peeling baffle 20a faces against rotating direction of the fixing roller 601 and is close to the fixing roller 601.

FIG. 4 is a schematic view showing an example of the fixing device (a type using a soft roller and a heat roller) used in the present invention.

The fixing device 10 shown in FIG. 4 is the type using the soft roller and the heat roller, which ensures a fixing nip while preventing the transfer material from winding to the roller, and provides excellent image quality. The fixing device 10 includes, a heat roller 601 as a heating member, a pressing roller 17b as a soft roller member and the halogen lamp 14 as a heat source inside the heat roller 601.

In the fixing device 10, a nip section N is formed between the heat roller 601 and the pressing roller 17b, and when heat and pressure are applied through the nip section N, a toner image is fixed on the transfer material P. Herein, a halogen lamp (not shown) may also be provided as a heat member inside the pressing soft roller.

The heat roller 601 including a halogen heater 14 inside as heating device is a hard roller having a major diameter of 50-80 mm. The hard roller has a metal base and a releasing layer provided thereon, wherein the metal base is, for example, a cylindrical metal pipe 171a containing aluminum and having a wall thickness of 5 to 20 mm, and the releasing layer 173a provided on the surface of the metal pipe 171a is formed by applying PFA (perfluoroalkoxy) or using a PFA tube and has a thickness of 5-30  $\mu$ m.

The heat roller 601 is independently driven by actuating motor Ma through a reduction gear assembly Gka.

The pressing roller 17b as pressing device includes a cylindrical metal pipe 171b, a rubber layer 172b and a releasing layer 173b. The cylindrical metal pipe 171b is made of, for example, iron and has a wall thickness of 5-10 mm. The rubber layer 172b is formed on the cylindrical metal pipe 171b and made of a soft rubber, for example, a silicone rubber of the thickness of 3-15 mm, the rubber exhibiting the strength of 30Hs to 50Hs (A-type rubber strength in JIS). The releasing layer 173b is formed on the rubber layer 172b, by applying, for example, PFA or using, for example, a PFA tube. The thickness of the releasing layer 173b is preferably 15-100  $\mu$ m. Thus prepared pressing roller 17b is a soft roller having a major diameter of 50-80 mm. The pressing roller 17b is also independently driven by an actuating motor Mb through a reduction gear assembly Gkb.

On a circumference of the pressing roller 17b, a supplementary roller 17c having a halogen lamp Hla inside as a

heating member is provided on the upstream of nip section N of the heat roller 601 and the pressing roller 17b.

The supplementary roller 17c has a metal pipe 171c and a halogen lamp Hla, wherein the metal-pipe 171c is a cylindrical core metal having a major diameter of 1 to 3 mm and provided thereon a PFA (perfluoroalkoxy) coating, and the halogen lamp Hla is provided inside of the metal pipe 171c.

The supplementary roller 17c is pressed onto the pressing roller 17b with a spring (not shown in the figure) and driven along with the rotation of the pressing roller 17b.

The toner image or the toner color image formed on the recording paper (transfer material P) is fixed at the convex curved nip section N formed between the heat roller 601 which is a hard roller and the pressing roller 17b which is a soft roller.

A contacting or non-contacting temperature sensor TS1 to the heat roller 601 is provided to control the temperature of the heat roller 601. The temperature of the supplementary roller 17c is controlled using a contacting or non-contacting temperature sensor TS2 to the supplementary roller 17c.

## EXAMPLES

The present invention will be specifically described with reference to examples. However, the embodiments of the present invention are not limited thereto.

### <Preparation of Ester Compounds Having a Specified Structure>

30 Polycarboxylic acids and long-chain aliphatic alcohols having 10 through 30 carbon atoms were subjected to the dehydration-condensation reaction to produce the above described compounds (1-1) (1-7), (2-1)-(2-7) and (3-1)-(3-16).

The reaction was carried out under nitrogen atmosphere at 220° C. for 8 hours, and after the reaction was completed, the resulting system was cooled down to 80° C. at a cooling rate of 20° C./min, being subjected to the neutralization reaction using a potassium hydroxide solution, and then subjected to cleaning, dehydration, and filtering to obtain the above compounds.

40 Compounds (3-1), (3-8), (3-9), (3-12) and (3-16) as the compounds represented by Formula (3), compounds (1-1)-(1-5) and (1-7) as the compounds represented by Formula (1) and compound (2-1) as the compounds represented by Formula (2) were weighed as shown in Table 1 and mechanically mixed to prepare ester mixtures A-G.

### <Preparation of Toners>

#### (Preparation of Colored Particle Bk1)

##### (1) Preparation of Low Molecular Weight Latex:

50 Into a 1 liter four-necked flask equipped with a mixer, a cooling tube and a temperature sensor, charged were 509.83 g of styrene, 88.67 g of n-butyl acrylate, 34.83 g of methacrylic acid, 21.83 g of tert-dodecyl mercaptan, and 66.7 g of the ester mixture (A). With the inner temperature raised to 80° C., the contents of the flask were stirred until the ester mixture (A) was dissolved and then the temperature was kept constant. On the other hand, a surfactant solution in which 1.0 g of sodium dodecyl benzenesulfonate was dissolved in 2700 ml of deionized water was similarly heated so that the inner temperature was raised to 80° C. and kept constant. With stirring, the surfactant solution kept at 80° C. was added with the monomer solution with the ester mixture (A) dissolved therein, and the resulting liquid was emulsified using an ultrasonic emulsifying device to obtain an emulsified liquid. Next, into a 5-liter four-necked flask equipped with a mixer, a

cooling tube, a nitrogen introduction tube and a temperature sensor, the emulsified liquid was charged, and under a flow of nitrogen with the inner temperature kept at 70° C., the content of the flask was added with a polymerization initiator solution in which 7.52 g of ammonium persulfate was dissolved in 500 ml of deionized waster with stirring, and polymerization was carried out for 4 hours, followed by cooled down to a room temperature and filtered to obtain a latex. After the reaction, the polymerization residue was not observed and stable latex was obtained. This was represented as "latex (L-1)".

For the obtained "latex (L-1)", the number average primary particle diameter was measured using an electrophoresis light scattering photometer "ELS-800" (manufactured by Otsuka Electronics Co., Ltd.) and determined to be 125 nm. The glass transition temperature was measured by DSC and determined to be 58° C. Further, the solid content of the above latex measured based on the dry weighing method by the rack drying was 20% by weight.

(2) Preparation of High Molecular Weight Latex:

Into a 1 liter four-necked flask equipped with a mixer, a cooling tube and a temperature sensor, charged were 92.47 g of styrene, 30.4 g of n-butyl acrylate, 3.80 g of methacrylic acid, 0.12 g of tert-dodecyl mercaptan, and 13.34 g of the ester mixture (A), with the inner temperature raised to 80° C., the contents of the flask were stirred until the ester mixture (A) was dissolved and then the temperature was kept constant. On the other hand, a surfactant solution in which 0.27 g of sodium dodecylbenzenesulfonate was dissolved in 540 ml of deionized water was similarly heated so that the inner temperature was raised to 80° C. and kept constant. With stirring, the surfactant solution kept at 80° C. was added with the monomer solution with the ester mixture (A) dissolved therein, and the resulting solution was emulsified using an ultrasonic emulsifying device to obtain an emulsified liquid. Next, into a 5-liter four-necked flask equipped with a mixer, a cooling tube, a nitrogen introduction tube and a temperature sensor, the emulsified liquid was charged, and under a flow of nitrogen with the inner temperature thereof kept at 70° C., the content of the flask was added with a polymerization initiator solution in which 0.27 g of ammonium persulfate was dissolved in 100 ml of deionized waster, with stirring. Polymerization was carried out for 4 hours followed by cooled down to a room temperature and filtered to obtain a latex. After the reaction, the polymerization residue was not observed and stable latex was obtained. This was represented as "latex (H-1)".

For the obtained "latex (H-1)", the number average primary particle diameter was measured using the electrophoresis light scattering photometer "ELS-800" (manufactured by Otsuka Electronics Co., Ltd.) and determined to be 108 nm. The glass transition temperature was measured by DSC and determined to be 59° C. Further, the solid content of the latex measured based on the dry weighing method by the rack drying was 20% by weight.

(3) Preparation of Colored Particle Bk:

Charged into a 5-liter four-necked flask equipped with a mixer, a cooling tube and a temperature sensor were 250 g of the latex (H-1), 1000 g of the latex (L-1), 900 ml of deionized water, and a carbon black dispersion containing 20 g of carbon black "REGAL 330R" (manufactured by Cabot Corp.) dispersed in a surfactant solution (a solution in which 9.2 g of sodium dodecylsulfate was dissolved in 160 ml of deionized water), and, with stirring, the contents of the flask were added with 5N sodium hydroxide solution to adjust the pH to 10. Further, with stirring, the resulting solution was added with a solution with 28.5 g of magnesium chloride 6hydrate dissolved in 1000 ml of deionized water under the room temperature, followed by raising the inner temperature to 95° C. While the inner temperature was kept at 95° C., the volume median diameter ( $D_{v50}$ ) was measured using "COULTER

MULTISIZER III" (manufactured by BECKMAN COULTER, Inc.). At the time when the particle diameter was 6.5  $\mu$ m, a solution with 80.6 g of sodium chloride dissolved in 700 ml of deionized water was added, and the reaction was further continued for 6 hours with the inner temperature kept at 95° C. After the reaction was completed, the obtained dispersion of the associated particles (95° C.) was cooled to 45° C. in 10 minutes (cooling speed=5° C./min.). The associated particles (colored particle Bk) prepared as described above were filtered, cleaned through repeating resuspension to deionized water and filtering, and then dried to obtain colored particle Bk. This was represented as "colored particle Bk1". The median diameter and CV value of "colored particle Bk1", were measured by "COULTER MULTISIZER III" (manufactured by BECKMAN COULTER, Inc.), and determined to be as follows: volume median diameter ( $D_{v50}$ )=6.5  $\mu$ m, CV value=18.2%.

(Preparation of Colored Particle Bk2)

"Colored particle Bk2" was prepared in the same manner as colored particle Bk1 except that 100 g of the ester mixture (A) was used in the preparation of low molecular weight latex instead of 66.7 g of the ester mixture (A) used in the preparation of the colored particle Bk1.

(Preparation of Colored Particle Bk3)

"Colored particle Bk3" was prepared in the same manner as colored particle Bk1 except that 20.0 g of the ester mixture (A) was used in the preparation of low molecular weight latex instead of 66.7 g of the ester compound (1) used in the preparation of the colored particle Bk1.

(Preparation of Colored Particle Bk4)

"Colored particle Bk4" was prepared in the same manner as colored particle Bk1 except that the ester mixture (B) was used instead of the ester mixture (A).

(Preparation of Colored Particle Bk5)

"Colored particle Bk5" was prepared in the same manner as colored particle Bk1 except that the ester mixture (C) was used instead of the ester mixture (A).

(Preparation of Colored Particle Bk6)

"Colored particle Bk6" was prepared in the same manner as colored particle Bk1 except that the ester mixture (D) was used instead of the ester mixture (A).

(Preparation of Colored Particle Bk7)

"Colored particle Bk7" was prepared in the same manner as colored particle Bk1 except that the ester mixture (E) was used instead of the ester mixture (A).

(Preparation of Colored Particle Bk8)

"Colored particle Bk8" was prepared in the same manner as colored particle Bk1 except that the ester mixture (F) was used instead of the ester mixture (A).

(Preparation of Colored Particle Bk9)

"Colored particle Bk9" was prepared in the same manner as colored particle Bk1 except that the ester mixture (G) was used instead of the ester mixture (A).

(Preparation of Colored Particle Bk10)

"Colored particle Bk10" was prepared in the same manner as colored particle Bk1 except that the ester compound (3-12) was used instead of the ester mixture (A).

(Preparation of Colored Particle Bk11)

"Colored particle Bk11" was prepared in the same manner as colored particle Bk1 except that Carnauba wax was used instead of the ester mixture (A).

(Preparation of Colored Particles C1-C11)

"Colored particles C1-C11" were prepared in the same manner as colored particles Bk1-Bk11 except that 10 g of C. I. Pigment Blue 15:3 was used instead of 20 g of REGAL 330R (manufactured by Cabot Corp.).

## (Preparation of Colored Particles M1-M11)

"Colored particles M1-M11" were prepared in the same manner as colored particles Bk1-Bk11 except that 17 g of C. I. Pigment Red 122 was used instead of 20 g of REGAL 330R (manufactured by Cabot Corp.).

## (Preparation of Colored Particles Y1-Y11)

"Colored particles Y1-Y11" were prepared in the same manner as colored particles Bk1-Bk11 except that 18 g of C. I. Pigment Yellow 17 was used instead of 20 g of REGAL 330R (manufactured by Cabot Corp.).

The mixtures of the ester compounds used for the preparation of colored particles Bk1-Bk11, volume median diameters, CV values are listed in Table 1.

Fixing rate: 280 mm/sec (about 50 A4 size sheets per minute when fed parallel to the short edge (long edge feed))

Heat roller surface temperature: arbitrary settable in the range of 90-240° C.

## 5 &lt;Evaluation&gt;

Using the above evaluation device, each of the toners and each of the developers were sequentially filled to carry out printing, and the evaluation was carried out on the following items.

10

## &lt;&lt;Evaluation of the Fixable Temperature&gt;&gt;

The temperature of the transfer material immediately after discharged from the heat roll was varied from 90-200° C. at

TABLE 1

| Colored particle No. | Ester mixture No. | Ester mixture having specified structure |              |                     |              |                     |              | Median CV value (%) |          |
|----------------------|-------------------|------------------------------------------|--------------|---------------------|--------------|---------------------|--------------|---------------------|----------|
|                      |                   | Amount (g)                               | Compound No. | Mixing ratio (wt %) | Compound No. | Mixing ratio (wt %) | Compound No. | Mixing ratio (wt %) |          |
| Bk1                  | A                 | 66.7                                     | 3-12         | 60                  | 1-2          | 40                  | —            | 0                   | 6.4 18.2 |
| Bk2                  | A                 | 100.0                                    | 3-12         | 90                  | 1-2          | 10                  | —            | 0                   | 6.6 17.8 |
| Bk3                  | A                 | 20.0                                     | 3-12         | 60                  | 1-2          | 40                  | —            | 0                   | 6.4 18.0 |
| Bk4                  | B                 | 66.7                                     | 3-1          | 60                  | 1-2          | 30                  | 2-1          | 10                  | 6.5 18.3 |
| Bk5                  | C                 | 66.7                                     | 3-12         | 60                  | 1-3          | 40                  | —            | 0                   | 6.4 18.5 |
| Bk6                  | D                 | 66.7                                     | 3-12         | 70                  | 1-4          | 30                  | —            | 0                   | 6.5 18.1 |
| Bk7                  | E                 | 66.7                                     | 3-16         | 80                  | 1-1          | 20                  | —            | 0                   | 6.3 18.3 |
| Bk8                  | F                 | 66.7                                     | 3-8          | 70                  | 1-6          | 30                  | —            | 0                   | 6.2 17.8 |
| Bk9                  | G                 | 66.7                                     | 3-9          | 60                  | 1-7          | 40                  | —            | 0                   | 6.6 17.5 |
| Bk10                 | —                 | 66.7                                     | 3-12         | 100                 | —            | 0                   | —            | 0                   | 6.4 17.9 |
| Bk11                 | —                 | 66.7                                     | Carnauba wax | 100                 | —            | 0                   | —            | 0                   | 6.5 17.6 |

The data for Colored particles C1-C11, M1-M11 and Y1-Y11 were similar to those for colored particles Bk1-Bk11, therefore, listing was abbreviated.

## (External Additive Treatment of the Colored Particles)

Next, each of the colored particles prepared as described above was added with 1% by weight of hydrophobic silica (the number average primary particle diameter: 12 nm, the hydrophobic ratio=68) and 1% by weight of hydrophobic titanium oxide (the number average primary particle diameter: 20 nm, the hydrophobic ratio=63), and was mixed using "HENSCHEL MIXER" (manufactured by Mitsui Miike Co., Ltd.) for 10 minutes. Subsequently, coarse particles were removed using a sieve of aperture 45  $\mu\text{m}$  to prepare toners Bk1-Bk11, C1-C11, M1-M11 and Y1-Y11. These were referred to as Examples Bk1-Bk9, Examples C1-C9, Examples M1-M9 and Examples Y1-Y9; and Comparative examples Bk1 and Bk2, Comparative examples C1 and C2, Comparative examples M1 and M2 and Comparative examples Y1 and Y2.

## &lt;Preparation of Developers&gt;

Each of the toners prepared as described above was mixed with a ferrite carrier coated with silicon resin and having volume median diameters ( $D_{V50}$ ) of 60  $\mu\text{m}$  so that the content of each of the toners was 6% by weight to prepare Developers Bk1-Bk11, Developers C1-C11, Developers M1-M11 and Developers Y1-Y11.

## &lt;Evaluation Device&gt;

The fixing device shown in FIG. 3 was mounted to the image forming apparatus described in FIG. 1 to be used as the evaluation device. Incidentally, the fixing rate and the heat roller surface temperature were set as described below.

35

intervals of every 10° C. to produce fixed images under a condition of 20° C. and 50% RH. A4-size fine-quality paper (65 g/m<sup>2</sup>) was used as the transfer material.

40

The fixable temperature was determined by evaluating the fixing strength of the obtained images with a mending tape stripping method described in "DENSHISYASHIN GIJYUTSU NO KISO TO OUYOU (Base and Application of Electrophotographic Technology): edited by Imaging Society of Japan" Chapter 9, Section 1.4. More specifically, the temperature of the transfer material surface was varied, and for each of the temperatures, a 2.54 cm square of fixed solid image with the toner amount of 0.6 mg/cm<sup>2</sup> was prepared, and the image densities of before and after the image stripping test using "Scotch Mending Tape" (manufactured by Sumitomo 3M Co., Ltd.) were measured, and the ratio of residual toner image was determined as the fixing ratio.

## 55 Tape Stripping Method:

(1) Measuring the absolute reflection density  $D_0$  of a 5 mm square black solid image.

(2) Lightly applying "Mending Tape" (equivalent to No. 810-3-12, manufactured by Sumitomo 3M Co., Ltd.).

(3) Rubbing the tape 3.5 times in both ways with the pressure of 1 kPa.

(4) Stripping the tape at the angle of 180° and with the strength of 200 g.

(5) Measuring the absolute reflection density  $D_1$  after stripping.

(6) Fixing ratio=100× $D_1/D_0$  (%)

The fixable temperature was defined as the lowest temperature which gave a fixing ratio of 90% or more.

Reflection density meter: RD-918 manufactured by GretagMacbeth was used for the image density measurement.

The temperature of the heat roller was set to 150° C.

Under a low-temperature and low-humidity condition (10° C., 20% RH), continuous printing was carried out on 1000 sheets of A3-size fine-quality paper (65 g/m<sup>2</sup>) with humidity controlled in the same environment, and a visual observation was made for both the images and the heat roller surface after completion of the 1000-sheet printing and an evaluation was made from the degree of the toner adhesion generated on the printed images and the heat roller surface.

The temperature of the transfer material surface just after discharged was around 100° C.

Evaluation Criteria:

A: No offset was observed on the heat roller and the image.

B: Offset was observed only on the heat roller while no offset was observed on the image; suitable for practical use.

C: Stain due to the offset was observed on the image: not suitable for practical use.

<<Image Evaluation>>

The fixing rate was set to 280 mm/sec, and the temperature of the heat roller was set to 150° C. so that the temperature of the transfer material surface was controlled to be around 100° C.

Under a condition of 20° C., 50% RH, 100,000 sheets of A3-size full color printing of which pixel density was 5%, on fine-quality paper (65 g/m<sup>2</sup>), were intermittently carried out, followed by being left overnight. Then, further printing was carried out and densities and fogs of the first printed image and the continuously printed 100th printed image were evaluated.

<Image Density>

The density of the black solid image portion was evaluated based on the relative density (the density of the transfer material without being printed was set to 0.0). Reflection density meter "RD-918" (manufactured by GretagMacbeth) was used for the measurement.

<Fog>

The fog density of the white portion of the print transfer material was expressed as a relative density when the image density of white background portion of unused transfer material was set to 0.000. Reflection density meter "RD-918" (manufactured by GretagMacbeth) was used for the measurement.

The evaluation results were summarized in Table 2.

As is apparent from Table 2, any of Examples Bk1-Bk9, Examples C1-C9, Examples M1-M9 and Examples Y1-Y9 exhibited excellent results in any evaluation items, while Comparative examples Bk1 and Bk2, Comparative examples C1 and C2, Comparative examples M1 and M2 and Comparative examples Y1 and Y2 showed problems in some of the evaluation items.

What is claimed is:

1. An electrostatic image developing toner comprising a binder resin and a colorant, wherein the toner comprises a mixture of:

- (i) a compound represented by Formula (3); and
- (ii) at least one of the compounds represented by Formula (1) or (2):



wherein, R<sub>1</sub>, R<sub>2</sub> and R<sub>3</sub> each independently represent an alkyl group having 10 to 30 carbon atoms and the alkyl group may have a substituent;



wherein, R<sub>4</sub> and R<sub>5</sub> each independently represent an alkyl group having 10 to 30 carbon atoms and the alkyl group may have a substituent; and



wherein, X represents H or —CO—R<sub>9</sub>, R<sub>9</sub> represents an alkyl group having 1-4 carbon atoms, where the alkyl group may have a substituent, and R<sub>6</sub>, R<sub>7</sub>, and R<sub>8</sub> each independently

TABLE 2

|         |      | Colored<br>particle No. |     | Fixable<br>temperature<br>(°C.) | Fixing<br>offset | Image<br>density<br>1st/100th | Fog<br>1st/100th      |
|---------|------|-------------------------|-----|---------------------------------|------------------|-------------------------------|-----------------------|
| Ex. 1   | Bk1  | Y1                      | M1  | C1                              | 110              | A                             | 1.41/1.40 0.001/0.001 |
| Ex. 2   | Bk2  | Y2                      | M2  | C2                              | 110              | A                             | 1.41/1.41 0.001/0.001 |
| Ex. 3   | Bk3  | Y3                      | M3  | C3                              | 120              | B                             | 1.41/1.41 0.001/0.001 |
| Ex. 4   | Bk4  | Y4                      | M4  | C4                              | 110              | A                             | 1.40/1.40 0.001/0.001 |
| Ex. 5   | Bk5  | Y5                      | M5  | C5                              | 110              | A                             | 1.42/1.42 0.001/0.001 |
| Ex. 6   | Bk6  | Y6                      | M6  | C6                              | 110              | A                             | 1.41/1.41 0.001/0.001 |
| Ex. 7   | Bk7  | Y7                      | M7  | C7                              | 110              | A                             | 1.41/1.41 0.001/0.001 |
| Ex. 8   | Bk8  | Y8                      | M8  | C8                              | 110              | A                             | 1.41/1.40 0.001/0.001 |
| Ex. 9   | Bk9  | Y9                      | M9  | C9                              | 110              | A                             | 1.41/1.41 0.001/0.001 |
| Comp. 1 | Bk10 | Y10                     | M10 | C10                             | 140              | C                             | 1.41/1.30 0.006/0.007 |
| Comp. 2 | Bk11 | Y11                     | M11 | C11                             | 150              | C                             | 1.38/1.21 0.007/0.010 |

Ex.: Example,

Comp.: Comparative example

represent an alkyl group having 10 to 30 carbon atoms, where the alkyl group may have a substituent.

2. The toner of claim 1, wherein the weight content of the mixture is 1 to 15% by weight of the toner.

3. The toner of claim 2, wherein (i) the compound represented by Formula (3) is contained in an amount of 50% or more by weight of the compounds represented by Formula (3) and (ii) at least one of the compound represented by Formula (1) or (2).

4. The toner of claim 1, wherein the weight content of the mixture is 3 to 12% by weight of the toner.

5. The toner of claim 1, wherein (i) the compound represented by Formula (3) is contained in an amount of 50% or more by weight of the compound represented by Formula (3) and (ii) at least one of the compounds represented by Formula (1) or (2).

6. The toner of claim 1, having a volume median diameter ( $D_{V50}$ ) in the range of 3 to 9  $\mu\text{m}$ .

7. The toner of claim 1, wherein a CV value in volume particle size distribution of the toner is not more than 20%.

8. The toner of claim 1, wherein the mixture comprises at least one of the following compounds (1-1) to (1-7), (2-1) to (2-7), and comprises at least one of the following compounds (3-1) to (3-16):



(1-1)



(1-2)



(1-3)



(1-4)



(1-5)



(1-6)



(1-7)



(2-1)



-continued

(2-2)



(2-3)



(2-4)



(2-5)



(2-6)



(2-7)



(3-1)



(3-2)



(3-3)



(3-4)



(3-5)



(3-6)



(3-7)

-continued



-continued

- (3-8) 5       $\text{C}_4\text{H}_9\text{COO}-\text{C}(\text{CH}_2\text{COOC}_{22}\text{H}_{45})(\text{CH}_2\text{COOC}_{22}\text{H}_{45})-\text{COOC}_{22}\text{H}_{45}$
- (3-9) 10     9. The toner of claim 8, wherein the weight content of the mixture is 3 to 12% by weight based on the total weight of the toner and the toner has a volume median diameter ( $D_{v,50}$ ) in the range of 3 to 9  $\mu\text{m}$ .
- (3-10) 15     10. The toner of claim 9, wherein (i) the compound represented by Formula (3) is contained in an amount of 50% or more by weight of the compound represented by Formula (3) and (ii) at least one of the compounds represented by Formula (1) or (2).
- (3-11) 20     11. The toner of claim 1, wherein the mixture exists in the toner particle as micro domains.
- (3-12) 25     12. The toner of claim 1, wherein (i) the compound represented by Formula (3) is contained in an amount of 60 to 98% by weight of the compounds represented by Formula (3) and (ii) the compound represented by at least one of Formulas (1) and (2).
- (3-13) 30     13. The toner of claim 1, wherein (i) the compound represented by Formula (3) is contained in an amount of 50 to 95% by weight of the compounds represented by Formula (3) and (ii) at least one of the compounds represented by Formula (1) or (2).
- (3-14) 35     14. An image forming method comprising: developing a latent image with a toner as defined in claim 1 so as to form a toner image.
- (3-15) 40     15. The image forming method of claim 14, further comprising fixing the toner image on an image forming material by passing between a first rotating member and a second rotating member, wherein at least one of the first and second rotating members gives heat to the toner image.
16. The image forming method of claim 15, wherein the first rotating member is a roller and is provided with a heat source inside of the roller.
17. The image forming method of claim 16, wherein the second rotating member includes a roller or an endless belt.

\* \* \* \* \*